# EUROPEAN PATENT SPECIFICATION

(11) **EP 0 124 360 B1**
(45) Date of publication and mention of the grant of the patent: **06.07.1988**
(21) Application number: 84302833.3
(22) Date of filing: 26.04.1984
(51) Int. Cl.: G09F 3/02, G09F 3/10

(54) **Printing bar-code labels**
Drucken von Strichcode-Etiketten
Impression d'étiquettes de codage en forme de barres

(30) Priority: 28.04.1983 JP 64286/83
(43) Date of publication of application: 07.11.1984
(73) Proprietor: KUREHA KAGAKU KOGYO KABUSHIKI KAISHA, Tokyo 103 (JP)
(72) Inventor: Okada, Yoshio, Iwaki-shi Fukushima-ken (JP); Ahiko, Nobuo, Iwaki-shi Fukushima-ken (JP); Igarashi, Yuriko, Iwaki-shi Fukushima-ken (JP); Suzuki, Masayasu, Iwaki-shi Fukushima-ken (JP)
(74) Representative: Myerscough, Philip Boyd

(56) References cited:
- DE-A- 2 325 567
- DE-A- 2 407 822
- DE-A- 2 518 871
- FR-A- 1 439 278
- US-A- 3 043 732

## Description

This invention relates to printing material sets for preparing bar-code labels by pressure-sensitive printing.

Recently, bar-code labels have become utilized in large quantities in which plural bar-codes are printed on the bar-code labels. The plural bar-codes indicated numeral letters which show information such as a name, a price and a weight of a commodity or an article. The bar-code labels are utilized in the statistical analysis of information concerning the distribution of the commodities or the articles.

Hitherto, as a process for preparing the bar-code labels, several methods of printing with carbon papers, thermosensitive papers or magnetic tapes have been devised while utilizing various types of simplified printers respectively suitable for the materials to be printed other than the transfer-ink printing method on an ordinary sheet of paper. However, the printing method such as an ink-printing method causes a stain on the hand when changing the ink-roll or an unevenness of the printed image of the bar-codes. Further, special means are necessary to stabilize the printed image of the bar-codes against friction. In the thermosensitive printing method, there are many occasions of pollution of the finished image of the bar-codes by after-color development due to heating because both the color-developer and the color-former exist on the surface of the label after thermal printing..In the case of using a carbon-paper, the transfer-printed pigment and wax adhere on the finished label. Therefore, the distinctness of the image of the bar-codes is apt to be reduced by heat and friction.

Every one of the defects mentioned above is a cause of reduction of the precision with which bar-codes are read by a light pen. The reduction is particularly noticeable in the case where the bar-codes are printed on a sheet of paper for the label on occasion and then the bar-code label is -adhered onto commodities or articles on occasion.

DE-A-2407822 discloses a self-adhesive record carrier, such as an adhesive label, composed of a base-paper, an adhesive layer on the back, a non-stick silicone layer or the like and a disposable backing sheet. Pressure-sensitive microcapsules contain a colour former are provided together with a colour-generating reagent layer. The base paper or the backing sheet of the adhesive label contains at least one of the two layers. The record carrier is described as for use in a factory. For example, an original carrier in front < can be used as an order confirmation, the adhesive label can be used as an information carrier for goods during the production sequence, storage and transport, and further duplicate carriers can be used for controlling production, storage and transport, as a consignment note or the like. There is no mention of bar-code labels.

According to this invention, there is provided a printing material set for preparing bar-code labels by pressure-sensitive printing, comprising an adhesive label which comprises a base paper, an adhesive layer and a backing sheet and, on top, a carrier which comprises a base which carries a coating of microcapsules on its back; characterised in that the set comprises
(a) a printing tape composed of a plastic film of a thickness of 30 µm or less as the base of the carrier, the microcapsules containing a solution of a colored dyestuff selected from a monoazo compound, a bisazo compound, a metal-complex salt of a monoazo compound, an anthraquinone compound, a phthalocyanine compound and a triarylmethane compound, and
(b) a tape as the backing sheet onto which, as the base paper, papers for the bar-code labels are removably attached at predetermined intervals by adhesive.

The invention also provides a method for preparing a bar-code label, which method comprises providing a printing set comprising an adhesive label which comprises a base paper, an adhesive layer and a backing sheet and, on top, a carrier which comprises a base which carries a coating of microcapsules on its back; and pressing together the carrier an adhesive label to break the microcapsules therebetween, characterised in that the set comprises
(a) a printing tape composed of a plastic film of a thickness of 30 11m or less as the base of the carrier, the microcapsules containing a solution of a colored dyestuff selected from a monoazo compound, a bisazo compound, a metal-complex salt of a monoazo compound, an anthraquinone compound, a phthalocyanine compound and a triarylmethane compound, and
(b) a tape as the backing sheet onto which, as the base paper, papers for bar-code labels are removably attached at predetermined intervals by adhesive, and the printing tape and papers for the bar-code labels are pressed together such that the microcapsules which contact the papers for bar-code labels break so as to print bar-codes thereon.

This invention will be described with reference to Figures 1 and 2, in which
Figure 1 is a partial cross-section view of a printing material set of this invention, and
Figure 2 is a plane view of a bar-code label according to this invention.

Referring to Figure- 1 of the drawings, the printing material set for preparing bar-code labels by pressure-sensitive printing method of our invention, comprises a printing tape 1, microcapsule layer 2, bar-code label papers 3, an adhesive agent 4 and a stripping tape 5. The microcapsules of layer 2 are carried on the printing tape 1 and contain a solution of a colored dyestuff. The bar-code label papers 3 are provided when an adhesive agent 4 on the under surface thereof facing on the stripping tape 5. The bar-code label papers 3 are detachably adhered to the stripping tape 5 with the adhesive agent 4 at predetermined intervals.

The microcapsules of layer 2 are crushed by applying a pressure in printing operation and the solution of the colored dyestuff containing therein is flowed onto one of the bar-code label papers 3 to print bar-code on the bar-code label paper. The flowed solution of the colored dyestuff is immediately absorbed into the bar-code label paper and then fastened thereat. The colored dyestuff remains in a stable state after the evaporation of the solvent of the solution. Thereafter, the printed bar-code label paper, that is the bar-code label, is detached from the stripping tape 5 and then, is applied to a commodity or an article.

In the case of carrying out the pressure-sensitive printing method with the printing material set of this invention for printing the bar-codes, it is necessary that the microcapsules at the pressed portion are uniformly crushed thereat by the pressure of percussion of the printer. For that purpose, the printing tape 1 should not be destroyed by the pressure of percussion of the printer and should have a uniform thickness. As a material suitable for the purpose, the present invention utilises a plastic film of a thickness of 30 µm or less than 30 µm, preferably from 6 to 20 µm may be mentioned. For example, polyethylene film and polypropylene film may be mentioned.

As the microcapsules held on the inside surface of the printing tape 1, the microcapsules for preparing the pressure-sensitive recording paper may be used. Accordingly, the microcapsules according to this invention may be prepared by the conventional process for the preparation of microcapsules.

As the colored dyestuff contained in the microcapsules, a dyestuff having a large solubility in organic solvents is used. More specifically, the dyestuff is selected from monoazo compounds such as Oil Brown #125^{®} (manufactured by YAMAMOTO KAGAKU GOUSEI K.K.) and Oil Brown BG extra@ (manufactured by SHIRADO KAGAKU KENKYUSHO); bisazo compounds such as Orient Oil Black HBB^{@} (manufactured by ORIENT KAGAKU KOGYO K.K.), Oil Scarlet SN^{®} (manufactured by SHIRADO KAGAKU KENKYUSHO), and Oleosol Red BB@ (manufactured by SUMITOMO KAGAKU KOGYO K.K.); metal complex salts of monoazo compounds such as Aizen Metalon Red HGRS^{®} (manufactured by HODOGAYA KAGAKU KOGYO K.K.) and Aizen Spilon Orange GRH^{@} (manufactured by HODOGAYA KAGAKU KOGYO K.K.); anthraquinone compounds such as Orient Oil Violet #730^{@} (manufactured by ORIENT KAGAKU KOGYO K.K.), Iketon Violet extra@ (manufactured by IKEDA KAGAKU KOGYO K.K.), and Iketon Sudan Blue extra@ (manufactured by IKEDA KAGAKU KOGYO K.K.); triarylmethane compounds such as Methyl Violet 2B Base 125% (manufactured by NAC) and Victoria Blue F4R (manufactured by BASF A. G.); and phthalocyanine compounds such as Orient Oil Blue BO^{O} (manufactured by ORIENT KAGAKU KOGYO K.K.).

As the solvent for dissolving the colored dyestuff, for instance, alkylbenzenes such as toluene and xylene, diarylmethanes, diarylethanes, alkylbiphenyls, alkyl naphthalenes and the like may be mentioned.

The printing tape 1 having microcapsules is prepared by coating the suspension of the microcapsules in a latex such as vinylidene chloride on the tape for printing and drying the coated tape. Further, in order to hold the microcapsules on the inside surface of the tape for printing, the known methods may be adopted.

As the bar-code label papers 3, the conventional papers for a label may be adopted. For example, printing papers may be used for the bar-code label papers 3 and particularly, coated papers such as coat paper, art paper and synthetic paper may be preferably used for the bar-code label papers 3. The bar-code label papers are detachably adhered to the stripping tape 5 at a predetermined intervals via the adhesive agent 4 and the adhered bar-code label papers 3 are easily detached from the stripping tape 5 after printing. Accordingly, the detachability of the stripping tape 5 is necessary and the stripping tape 5 may be selected from the known materials as a stripping tape such as a coated paper, a laminated paper, a plastic film and a coated plastic film, which may be suitably selected according to the kind of the adhesive agent.

The adhesive agent 4 used herein may be selected from the known adhesive agents which can adhere pieces of papers 3 for printing the bar-codes to the commodity or the article. For example, as the adhesive agent 4, adhesive agents having pressure sensitivity such as an adhesive agents containing natural rubber, silicone polymer, acrylic polymer, acrylic copolymer, polyvinylpyrrolidone or copolymer of vinylpyrrolidone may be mentioned.

In the case where the bar-code labels are prepared by using laminated material of this invention, the printing may be carried out by applying a percussion pressure in a predetermined figure on the upper surface of the printing tape 1 thereby preparing a bar-code label with the bar-codes printed in a short time after applying the percussion pressure on the printing tape and evaporating the solvent of the solution. The obtained bar-codes on the label is fixed in a stable state, not to be stained by friction and to be maintained distinctly even after a few months.

This invention will be further illustrated by the following example which should not be construed as a limitation of this invention.

### Example

(i) Preparation of microcapsules containing dyestuff:
An aqueous solution of a melamine-formaldehyde prepolymer (hereinafter referred to as M4F prepolymer, M4F meaning that the molar ratio of formaldehyde to malamine is 4:1) was prepared by mixing 63 g of melamine and 162 g of aqueous 37% by weight solution of formaldehyde (hereinafter referred to as formalin) adjusted to pH of 9.0 with the addition of aqueous 2% by weight solution of sodium hydroxide, reacting melamine and formaldehyde at 70°C and adding 225 g of water just after the dissolution of melamine into the aqueous phase followed by stirring for 3 min.

Separately, an aqueous solution of a ureaformaldehyde prepolymer (hereinafter referred to as U 1.8 F prepolymer, U 1.8 F meaning that the molar ratio of formaldehyde to urea is 1.8) was prepared by mixing 60 g of urea and 146 g of formalin adjusted to pH of 8.5 with the addition of triethanolamine and reacting urea and formaldehyde at 70°C for one hour. The mixture of 20 g of a water-soluble cationic urea resin (Uramin^{@} P-1500, manufactured by Mitsui-Toatsu Co., Japan), 100 g of the M4F prepolymer, 50 g of the U 1.8 F prepolymer, 200 g of water and 1 g of triethanolamine was adjusted to pH of 5.2 by adding aqueous 10% by weight solution of citric acid, and then 3g of aqueous 10% by weight solution of sodium alkylbenzenesulfonate (Neopelex^{®}, manufactured by Kao-Atlas Co., Japan) was added to the mixture.

After adding a mixture of 3 g of dyestuff (Iketon Sudan Blue extra@), 50 g of the di-isopropyl naphthalene and 50 g of xylene further to the above- mentioned mixture, the whole system was subjected to homogenization in a homogenizer to be an emulsion containing droplets of 5 to 10 microns, in average diameter, and while maintain- ingthe temperature of the emulsion at 30°C it was gently stirred and the pH was adjusted to 3.8 with the addition of aqueous 10% by weight solution of citric acid. Then, after one hour, aqueous 10% by weight solution of citric acid was added again to the whole mixture to adjust the pH thereof to 3.0 and 100 g of water was added, and further by stirring the whole system as it was for 15 hours the microencapsulation was completed.

### (ii) Preparation of printing material set:

The prepared microcapsules were suspended in latex of vinylidene chloride and then, the suspension of the microcapsules was coated on the surface of polyethylene tape having 15 11m in thickness.

The coated polyethylene tape was set on pieces of paper for use in a bar-code label paper, which was previously laminated with stripping tape.

### (iii) Preparation of bar-code label:

The prepared printing material set as shown in Fig. 1 was printed by applying a percussion pressure and the printed images as shown in Fig. 2 were fixed on the surface of the bar-code label paper. The printed images were not stained by friction and were maintained distinctly even after a few months.

## Claims

1. A printing material set for preparing labels by pressure-sensitive printing, comprising an adhesive label which comprises a base paper, an adhesive layer and a backing sheet and, on top, a carrier which comprises a base which carries a coating of microcapsules on its back; characterised in that the set comprises
(a) a printing tape (1) composed of a plastic film of a thickness of 30 11m or less as the base of the carrier, the microcapsules (2) containing a solution of a colored dyestuff selected from a monoazo compound, a bisazo compound, a metal-complex salt of a monoazo compound, an anthraquinone compound, a phthalocyanine compound and a triarylmethane compound, and
(b) a tape (5) as the backing sheet onto which, as the base paper, papers (3) for bar-code labels are removably attached at predetermined intervals by adhesive (4).

2. A printing material set according to claim 1, wherein the microcapsules (2) are suitable for use in a pressure-sensitive recording paper.

3. A printing material set according to claim 1 or 2, wherein the colored dyestuff is dissolved in an organic solvent selected from alkylbenzenes, diarylmethanes, diarylethanes, alkylbiphenyls and alkylnaphthalenes.

4. A printing material set according to any one of the preceding claims wherein the plastic film is a polyethylene film or a polypropylene film.

5. A method for preparing a label, which method comprises providing a printing set comprising an adhesive label which comprises a base paper, an adhesive layer and a backing sheet and, on top, a carrier which comprises a base which carries a coating of microcapsules on its back; and pressing together the carrier and adhesive label to break the microcapsules therebetween, characterised in that the set comprises
(a) a printing tape (1) composed of a plastic film of a thickness of 30 ₁₁m or less as the base of the carrier, the microcapsules (2) containing a solution of a colored dyestuff selected from a monoazo compound, a bisazo compound, a metal-complex salt of a monoazo compound, an anthraquinone compound, a phthalocyanine compound and a triarylmethane compound, and
(b) a tape (5) as the backing sheet onto which, as the base paper, papers (3) for bar-code labels are removably attached at predetermined intervals by adhesive (4), and
the printing tape (1) and papers (3) for bar-code labels are pressed together such that the microcapsules (2) which contact the papers (3) for bar-code labels break so as to print bar-codes thereon.

6. A method according to claim 5 which further comprises, after pressing together the printing tape (1) and the bar-code label papers (3), removing the detachable tape (5) from the adhesive (4) on the under-surface of the bar-code label papers (3) and applying the bar-code label papers (3) to an article.

7. A method according to claim 5 or 6 wherein the microcapsules (2) are suitable for use in a pressure-sensitive recording paper.

8. A method according to any one of claims 5 to 7, wherein the dyestuff is dissolved in an organic solvent selected from alkylbenzenes, diarylmethanes, diarylethanes, alkylbiphenyls and alkylnaphthalenes.

9. A method according to any one of claims 5 to 8, wherein the plastic film is a polyethylene film or a polypropylene film.

## Patentansprüche

1. Druckmaterialeinheit zur Herstellung von Etiketten durch druckempfindliches Drucken aus einem Klebetikett aus einem Grundpapier, einer Klebschicht und einer Rückschicht und einem darüber befindlichen Träger aus einem Grundelement, das auf seiner Unterseite eine Beschichtung aus Mikrokapseln trägt, dadurch gekennzeichnet, daß die Einheit
(a) als Trägergrundelement ein Druckband (1) aus einer Kunststoffolie mit einer Dicke von 30 um oder weniger, wobei die Mikrokapseln (2) eine Lösung eines gefärbten Farbstoffs aus der eine Monoazoverbindung, eine Bisazoverbindung, ein Metallkomplexsalz einer Monoazoverbindung, eine Anthrachinonverbindung, eine Phthalocyaninverbindung und eine Triarylmethanverbindung umfassenden Gruppe enthalten, und
(b) als Rückschicht ein Band (5) auf dem als Grundpapier Strichcodeetikettenpapiere (3) in bestimmten Abständen mit einem Klebstoff (4) wiederentfernbar aufgebracht sind, umfaßt.

2. Druckmaterialeinheit nach Anspruch 1, dadurch gekennzeichnet, daß die Mikrokapseln (2) für die Verwendung in druckempfindlichen Aufzeichnungspapieren geeignet sind.

3. Druckmaterialeinheit nach Anspruch 1, dadurch gekennzeichnet, daß der gefärbte Farbstoff in einem organischen Lösungsmittel aus der Alkylbenzole, Diarylmethane, Diarylethane, Alkylbiphenyle und Alkylnaphtaline umfassenden Gruppe gelöst ist.

4. Druckmaterial nach einem dervorangegangenen Ansprüche, dadurch gekennzeichnet, daß die Kunststoffolie aus Polyethylen oder Polypropylen besteht.

5. Verfahren zur Herstellung eines Etiketts durch Vorsehen einer Druckeinheit aus einem Klebetikett aus einem Grundpapier, einer Klebschicht und einer Rückschicht und einem darüber befindlichen Träger aus einem Grundelement, das auf seiner Unterseite eine Beschichtung aus Mikrokapseln trägt und Aufeinanderdrücken des Trägers und des Klebetiketts zum Aufbrechen der dazwischenliegenden Mikrokapseln, dadurch gekennzeichnet, daß die Einheit
(a) als Trägergrundelement ein Druckband (1) aus einer Kunststoffolie mit einer Dicke von 30 um oder weniger, wobei die Mikrokapseln (2) eine Lösung eines gefärbten Farbstoffs aus der eine Monoazoverbindung, eine Bisazoverbindung, ein Metallkomplexsalz einer Monoazoverbindung, eine Anthrachinonverbindung, eine Phthalocyaninverbindung und eine Triarylmethanverbindung umfassenden Gruppe enthalten, und
(b) als Rückschicht ein Band (5), auf dem als Grundpapier für Strichcodeetikettenpapiere (3) in bestimmten Abständen mit einen Klebstoff (4) wiederentfernbar aufgebracht sind, umfaßt, und das Druckband (1) und die Strichcodeetikettenpapiere (3) aufeinandergedrückt werden, so daß die Mikrokapseln (2), die mit den Strichcodeetikettenpapieren (3) in Kontakt kommen, unter Bildung von dadurch aufgedruckten Strichcoden aufbrechen.

6. Verfahren nach Anspruch 5, dadurch gekennzeichnet, daß man weiterhin nach dem Aufeinanderdrücken des Druckbandes (1) und der Strichcodeetikettenpapiere (3) das abtrennbare Band (5) von dem Klebstoff (4) auf der unteren Oberfläche des Strichcodeetikettenpapiers (3) entfernt und die Strichcodeetikettenpapiere (3) auf einen Artikel aufbringt.

7. Verfahren nach Anspruch 5 oder 6, dadurch gekennzeichnet, daß die Mikrokapseln (2) zur Verwendung in druckempfindlichen Aufzeichnungspapieren geeignet sind.

8. Verfahren nach einem der Ansprüche 5 bis 7, dadurch gekennzeichnet, daß der Farbstoff in einem organischen Lösungsmittel aus der Alkylbenzole, Diarylmethane, Diarylethane, Alkylbiphenyle und Alkylnaphthaline umfassenden Gruppe gelöst ist.

9. Verfahren nach einem der Ansprüche 5 bis 8, dadurch gekennzeichnet, daß die Kunststoffolie aus Polyethylen oder Polypropylen besteht.

## Revendications

1. Ensemble formant matériau d'impression pour préparer des étiquettes par impression sensible à la pression, comportant une étiquette adhésive qui comprend un papier de base, une couche adhésive et une feuille au verso et, sur le dessus, un support qui comprend une base qui porte, au verso, une enduction de microcapsules; caractérisé en ce que l'ensemble comporte
a) un ruban d'impression (1) composé d'un film plastique d'une épaisseur de 30 pm ou moins comme base du support, les microcapsules (2) contenant une solution d'un produit colorant coloré choisi parmi un composé monoazoïque, un composé diazoïque, un sel métallique complexe d'un composé monoazoïque, un composé d'anthraquinone, un composé de phthalocyanine et un composé de triarylméthane, et
b) comme feuille au verso, un ruban (5) sur lequel, comme papier de base, des papiers (3) pour étiquettes à codes à barres sont attachés de façon amovible, à des intervalles prédéterminés, par un adhésif (4).

2. Ensemble formant matériau d'impression selon la revendication 1, dans lequel les microcap- suies (2) conviennent pour emploi dans un papier support d'enregistrement sensible à la pression.

3. Ensemble formant matériau d'impression selon la revendication 1 ou 2, dans lequel le produit colorant coloré est dissous dans un solvant organique choisi parmi les alcoylbenzènes, les diarylméthanes, les diaryléthanes, les phényl-2 alcoyles et les alcoyl naphtalènes.

4. Ensemble formant matériau d'impression selon l'une quelconque des revendications précédentes, dans lequel le film plastique est un film de polyéthylène ou un film de polypropylène.

5. Procédé de préparation d'une étiquette, procédé qui comporte le fait de disposer d'un ensemble d'impression comportant une étiquette autocollante qui comprend un papier de base, une couche adhésive et une feuille au verso et, sur le dessus, un support qui comprend une base qui porte, au verso, une enduction de microcapsules; et de presser ensemble le support et l'étiquette autocollante pour briser entre eux les microcapsules, caractérisé en ce que l'ensemble comporte
a) un ruban d'impression (1) composé d'un film plastique d'une épaisseur de 30 pm ou moins comme base du support, les microcapsules (2) contenant une solution d'un produit colorant coloré choisi parmi un composé monoazoïque, un composé diazoïque, un sel métallique complexe d'un composé monoazoïque, un composé d'anthraquinone, un composé de triarylméthane, et
b) comme feuille au verso, un ruban (5) sur lequel, comme papier de base, des papiers (3) pour étiquettes à codes à barres sont attachés de façon amovible, à des intervalles prédéterminés, par un adhésif (4), et en ce que
on presse ensemble le ruban d'impression (1) et les papiers (3) pour étiquettes à codes à barres de façon que les microcapsules; (2) qui viennent au contact des papiers (3) pour étiquettes à codes à barres se brisent pour y imprimer des codes à barres.

6. Procédé selon la revendication 5, comportant en outre le fait, après avoir pressé ensemble le ruban d'impression (1) et les papiers (3) pour étiquettes à codes à barres, de détacher le ruban détachable (5) d'avec l'adhésif (4) qui se trouve à la surface inférieure des papiers (3) pour étiquettes à codes à barres et d'appliquer les papiers (3) pour étiquettes à codes à barres sur un article.

7. Procédé selon la revendication 5 _ou 6, dans lequel les microcapsules (2) conviennent pour emploi dans un papier support d'enregistrement sensible à la pression.

8. Procédé selon l'une quelconque des revendications 5 à 7, dans lequel le produit colorant coloré est dissous dans un solvant organique choisi par les alcoylbenzènes, les diarylméthanes, les diaryléthanes, les phényl-2 alcoyles et les alcoyl naphtalènes.

9. Procédé selon l'une quelconque des revendications 5 à 8, dans lequel le film plastique est un film de polyéthylène ou un film de polypropylène.
